

# United States Patent

(11) 3,607,612

[72] Inventor **Robert L. Hudson**  
Saverna Park, Md.  
[21] Appl. No. **836,172**  
[22] Filed **June 24, 1969**  
[45] Patented **Sept. 21, 1971**  
[73] Assignee **Esso Research and Engineering Company**

2,313,757 3/1943 Matheson et al. .... 260/45.85  
2,921,044 1/1960 Coover, Jr. .... 260/878  
2,976,259 3/1961 Hardy et al. .... 260/31.8 G

*Primary Examiner*—Robert F. Burnett  
*Assistant Examiner*—Linda M. Carlin  
*Attorney*—Karl W. Flocks

(54) **SARAN RIBBON FOR DRY-CLEANABLE  
TEXTILES**  
10 Claims, No Drawings

(52) U.S. Cl. .... **161/181**,  
260/45.85, 260/878, 260/879, 260/884  
[51] Int. Cl. .... **C08f 45/36**,  
D01f 7/02  
[50] Field of Search ..... 161/172,  
181; 264/211; 260/31.8, 45.7, 45.85, 878, 879,  
884, 87.1, 87.7

(56) **References Cited**  
UNITED STATES PATENTS  
2,160,931 6/1939 Wileg ..... 260/87.1

**ABSTRACT:** Flat extruded saran filaments are provided for use in textile fabrics which may be dry cleaned in perchloroethylene without providing excessive shrinkage of the saran. The saran composition from which the flat filaments are formed must contain no more than 5 percent by weight of extractable organic additives based on the total quantity of the saran copolymer and the additives. The organic additives constitute a stabilizing plasticizer which is an ester of fumaric acid, maleic acid, itaconic acid oraconitic acid, and a light stabilizer; in addition, no more than about 0.5 percent of a nonextractable, primarily inorganic phosphate stabilizer is also used. The composition contains an additional quantity of about 5 percent of branched polyethylene.

**SARAN RIBBON FOR DRY-CLEANABLE TEXTILES**

The invention relates to saran ribbon for dry-cleanable textiles and, more particularly, to extruded saran monofilament of small thickness which is suitable for use in a fire-retardant textile fabric which may be dry cleaned in perchloroethylene without causing excessive shrinkage of the saran.

Saran is an old and well-known plastic which has a number of outstanding properties one of which is its noncombustability. Because of these properties its use has been suggested for many years in various areas and, among these, is its utilization as a textile fiber for use in various fabrics. Unfortunately, in addition to its outstanding properties, saran has a number of serious disadvantages; for example, it is extremely corrosive in the molten state and is difficult to handle and extrude. Until the present invention, it was impossible to successfully extrude saran filaments without at least about 7½ percent organic additives including plasticizers and stabilizers.

In recent years it has been suggested that saran filaments, particularly flat filaments, be used in the manufacture of various commercial fabrics, including draperies, because of the fireproof properties of the saran. Unfortunately, commercial draperies and other commercial fabrics must be capable of being dry cleaned and the common dry cleaning solvent in use today is perchloroethylene. It has been found that when saran fabrics are dry cleaned in perchloroethylene, the perchloroethylene extracts the organic additives, previously present in amount of 7½ percent to 10 percent, causing excessive shrinking of the saran. For this reason, it has not been commercially desirable to manufacture fabrics utilizing extruded saran filaments because of such excessive shrinkage after dry cleaning. The problem is particularly acute in the case of saran ribbon filaments, since these filaments have a very small dimension in one direction, i.e., they may be as little as 2 mils thick or even thinner, such small dimension permitting ready penetration of the perchloroethylene during dry cleaning, resulting in the extraction of almost all of the organic additives and the consequent excessive shrinkage of such filaments.

Many attempts have been made to solve the above problems such as through the selection of different plasticizers, different stabilizers, and various combinations of these materials. Nevertheless, in spite of all such attempts, it has heretofore been impossible to extrude such saran filaments without a minimum of 7½ percent of organic additive. Accordingly, before the present invention, the only successful approach to providing textile filaments intended for use in fabrics subjected to dry cleaning in perchloroethylene, was to form such filaments by methods other than extrusion, e.g. coagulation of a latex in film form followed by cutting the saran film into ribbon.

It is, accordingly, an object of the present invention to overcome the defects of the prior art, such as indicated above.

It is another object of the present invention to provide an extruded saran monofilament of small thickness which not only has the inherent fire retardant characteristics of saran, but which is also capable of being dry cleaned in perchloroethylene without causing excessive shrinkage.

It is another object of the present invention to provide a composition of saran which contains, at most, about 5 percent by weight of low molecular weight organic additives, which composition can be successfully extruded to form a commercial product.

It is another object of the present invention to provide a novel combination of ingredients including predominantly saran, which ingredients may be melt extruded to form a saran monofilament which is subsequently capable of being dry cleaned in perchloroethylene without causing excessive shrinkage thereof.

It is another object of the present invention to provide a flat saran monofilament which is satisfactorily stabilized, and yet is capable of being woven into fabrics without causing a buildup of stabilizer on the weaving equipment.

These and other objects and the nature and advantages of the instant invention will be more apparent from the following

description of an embodiment of the present invention, such description so fully revealing the general nature of the invention that others can, by applying current knowledge, readily modify such embodiment and/or adapt it for various applications without departing from the generic concept, such adaptations and modifications accordingly being intended to be part of the generic invention.

The composition used to form the extruded saran monofilament of small thickness of the disclosed embodiment, suitable for use in a fire retardant textile fabric, which fabric is capable of being dry cleaned in perchloroethylene, consists essentially of 100 parts by weight of a uniform saran copolymer of about 85 percent by weight vinylidene chloride and about 15 percent by weight vinyl chloride; about 0.0013 to 0.0075 moles of an organic stabilizing plasticizer which is an ester of fumaric acid, maleic acid, itaconic acid or aconitic acid; about 0.76 to 2.65 parts by weight of an organic light stabilizer, the total quantity of organic light stabilizer and organic stabilizing plasticizer being no greater than 5 percent by weight of the above-mentioned ingredients; about 0.16 to 0.51 parts by weight of a primarily inorganic phosphate, which may, however, have certain organic groups, which phosphate is not perchloroethylene extractable; about 3 to 9 parts by weight of branched polyethylene. The ribbon filaments produced preferably have a thickness of about 2 to 2.5 mils and a width of about 25 to 30 mils.

Saran itself is a well-known copolymeric plastic usually formed of approximately 85 percent vinylidene chloride and 15 percent vinyl chloride, although the proportion of vinyl chloride in the copolymer may lie anywhere in the range of from about 5 percent to about 15 percent, the remainder being vinylidene chloride. Many polymers of vinylidene chloride are described in the early U.S. Pat. Nos. 2,160,903; 2,160,904 and 2,160,931 through 2,160,948. The saran resins are generally crystalline, i.e., they have a relatively sharp melting point and may be extruded, quenched and oriented to form generally crystalline filaments. As pointed out in the Matlack et al. U.S. Pat. No. 2,605,244, the crystalline habit of saran makes compounding difficult since the polymer macromolecules prefer contact with each other and tend to reject foreign substances such as plasticizers and stabilizers.

The preferred saran copolymer for use in the present invention has a regular or uniform structure in the sense that the vinyl chloride groups are regularly spaced in the copolymer backbone without forming substantial blocks. This copolymer is preferably formed from a mixture of 85 percent by weight of vinylidene chloride and 15 percent by weight vinyl chloride. It has a melting point of slightly greater than 300° F.

In order to permit the extrusion of the saran, it is necessary to use at least a small quantity of plasticizer. The material so used in the present invention is a stabilizing plasticizer which is an ester of fumaric acid, maleic acid, itaconic acid, or aconitic acid. These known esters serve an important stabilizing function since, during extrusion of the molten saran, the polymer backbone undergoes dehydrohalogenation which results in color producing polyene segments. Since the dark color produced by such degradation is undesirable, the stabilizing plasticizers are provided to interrupt such color producing polymer segments.

This stabilization is accomplished by means of a Diels-Alder reaction between the maleate and the polyene segments produced by such degradation or dehydrohalogenation. Where fumarates are used, they isomerize to the cis-form and function in the same manner as the maleate. The aconitates and itaconates also react according to the Diels-Alder reaction with the polyene segments produced during extrusion.

Where the preferred stabilizing plasticizer, dioctyl fumarate, is used, it is preferably present in an amount of 1½ to 3½ percent by weight, based upon the weight of the composition exclusive of the polyethylene, and is most preferably present in an amount of 2.5 percent. However, because the alkyl group can vary considerably in the ester (it need not be dioctyl), it is desirable to express the proportion in moles per

hundred parts by weight of saran copolymer, and accordingly the preferred quantity of stabilizing plasticizer is 0.0045 to 0.0075 moles per 100 parts of saran copolymer.

While 1½ percent by weight or 0.0045 moles per 100 parts of copolymer is the preferred minimum, this may be reduced to as little as one-half percent by weight (considering dioctyl fumarate) or 0.0013 moles per 100 parts of copolymer. When the quantity of stabilizing plasticizer is so reduced, however, it is necessary to dry blend the primarily inorganic stabilizers, discussed below, with the copolymer or else use another liquid medium in which the inorganic stabilizer may be dispersed, and this provides for complicated processing.

It should be made clear that not all of the entire quantity of the above-mentioned stabilizing plasticizer will react with the saran during extrusion, but a small proportion will, the exact amount depending upon the amount of degradation produced during such extrusion. The remainder of the stabilizing plasticizers will serve a plasticizing function until the formed filaments are contacted with perchloroethylene during dry cleaning thereof, at which time the unreacted plasticizer will be extracted by the perchloroethylene.

As examples of further stabilizing plasticizers which may be used, there may be mentioned, besides dioctyl fumarate; triethylaconitate; tripropylaconitate; tributylaconitate; the methyl, benzyl and phenyl esters of aconitic acid; di-(2-benzoxy-ethyl) fumarate; benzyl esters of fumaric acid, maleic acid and itaconic acid; diethylitaconate; diallyl maleate; dibutyl maleate, etc.

Another perchloroethylene extractable material which must be included in the composition is an organic light stabilizer which is present in an amount of 0.76 to 2.65 parts by weight per 100 parts by weight of the saran copolymer. The preferred organic light stabilizer, which is an ultraviolet screen or absorbent, is 2-hydroxy-4-n-octyloxybenzophenone, and it is preferably present in an amount of 1.5 percent by weight based on the weight of saran and extractable organic additives. The above figure of 0.76 to 2.65 parts by weight of stabilizer based on 100 parts by weight of copolymer corresponds to 0.75 to 2½ percent by weight based on the composition including the copolymer and the extractable organic additives.

Such organic light stabilizer may be any 2-hydroxy-4-alkyloxybenzophenone up to and including stearyl (C18). The methyl, n-octyl, n-decyl and n-dodecyl are presently commercially available. Another effective light absorber which may be used is 2,4-dibenzoylresorcinol.

As indicated above, the total quantity of the organic light stabilizer and the organic stabilizing plasticizer must be no greater than 5 percent by weight based on the total quantity of the copolymer and such two organic additives. The 5 percent figure is obtained on the basis of commercial acceptance, since more than 5 percent by weight of such components will result in excessive shrinkage upon dry cleaning in perchloroethylene. The organic stabilizers and stabilizing plasticizers are, of course, compatible with the saran copolymer in the proportions delineated.

The presence of a primarily inorganic phosphate stabilizer in the composition is an important feature of the invention, and the proportions utilized are quite critical. While such phosphates have been known in the past to be necessary for use in saran copolymer compositions to provide adequate stabilization, it has previously been thought necessary to use quantities at least 1½ times as great as the maximum permissible according to the present invention. Accordingly, it was previously thought, when using the preferred inorganic phosphate stabilizer which comprises 88 percent by weight disodium phosphate and 12 percent by weight sodium pentacapryltripolyphosphate, that at least 0.75 percent by weight based on the total composition (exclusive of the polyethylene) was necessary. However, in accordance with the present invention it has now been found that at most 0.5 percent by weight may be tolerated (0.51 parts by weight per 100 parts of saran copolymer).

Thus, particularly in the case of flat, ribbon monofilaments, when the filaments are woven into textile fabrics, such as commercial drapery, it is found that when more than 0.51 parts by weight of the primarily inorganic phosphate stabilizer is used per 100 parts by weight of saran, a severe deposit problem on the weaving equipment is encountered. This buildup, called "loom-drip" is actually caused by filaments running over the loom and shuttle which have a tendency to scrape off the inorganic phosphate from the surface of the ribbon monofilaments. The problem is eliminated by reducing the quantity of inorganic phosphate stabilizer to 0.51 parts by weight or less per 100 parts of copolymer, and this surprisingly results in adequate stabilization, even after the organic stabilizers and plasticizers, exclusive of that portion of the stabilizing plasticizer which has reacted with the polyene portions of the copolymer, have been extracted by the perchloroethylene dry cleaning solvent.

The primarily inorganic phosphate stabilizer, as indicated above, remains with the copolymer even after dry cleaning in perchloroethylene i.e., it is perchloroethylene nonextractable. This material, which is an hydrochloric acid scavenger, is preferably present in an amount of 0.25 percent and its range of use is 0.15-0.50 percent by weight based on the composition exclusive of the polyethylene, or 0.16-0.51 parts by weight per 100 parts by weight of copolymer. The lower limit is critical since too little stabilizer will result in discoloration of the saran.

As indicated above, the preferred primarily inorganic phosphate is a blend of 88 percent disodium phosphate and 12 percent sodium pentacapryl tripolyphosphate, and this sold under the trade name "Victor 85X." Other suitable primarily inorganic phosphates which may be used in accordance with the present invention are sodium tripolyphosphate (DS 95), tetrasodium pyrophosphate, sodium hexametaphosphate, sodium barium phosphate, barium stearyl phosphate, barium lauryl phosphate, and sodium metaphosphate. Of course, various blends of these phosphates may also be used, or disodium phosphate or sodium pentacapryl tripolyphosphate may be used separately. It should be noted that not all inorganic phosphates are suitable, since some are not sufficiently reactive to scavenge the hydrochloric acid produced in the saran composition, while others are so reactive that they will scavenge the chlorine from the polymer which is, of course, highly undesirable.

In accordance with the present invention it has also been found to be particularly desirable, from a processing standpoint, to add an additional 3-9 percent, preferably 5 percent by weight, of a branched polyethylene to the composition. The addition of the branched polyethylene to the composition prevents the yarns from sticking together or welding in the quenching tank after extrusion or in the annealing tank after orientation. It is found that below about 3 percent polyethylene, some sticking will occur, while if more than 9 percent polyethylene is used, the nature of the extrusion is changed. Surprisingly, it is found that high density linear polyethylene is unsatisfactory for this purpose. Preferably, the branched polyethylene has a density of about 0.92, a melt index between about 1.5 and 4.0 and a melting point no greater than the melting temperature of the saran copolymer.

The preferred branched polyethylene used is du Pont's polyethylene TE-4275, which has a melt index of 3.7 a density of 0.923 and a melting point of 230°-250°F. The polyethylene is completely compatible with the saran in the proportions used. The filaments in accordance with the present invention are produced by extruding the composition through a die having an opening corresponding to the cross-sectional shape of the filament desired, namely, rectangular. The above-described components are mixed together, the primarily inorganic stabilizer being preferably initially dispersed in the organic stabilizing plasticizer, and the polyethylene being in fine particulate form, and the composition is passed into a heated screw extruder. The molten composition is forced through a plurality of rectangular orifices in the extrusion head of the ex-

truder and the filaments are pulled down through an airgap where partial orientation and modification to the cross sectional dimensions desired occur. The ribbons are then passed to an orientation zone where they are stretched approximately 4:1. Subsequent to orientation, an annealing is carried out at about 205° F. Where a slight degree of shrinkage is permitted.

The following specific example will further clarify the nature of the present invention without limitation:

A composition is provided by mixing 95.75 percent by weight of uniform saran of 85 percent vinylidene chloride and 15 percent vinyl chloride having a melting point of slightly greater than 300° F. with 2.5 percent by weight diethyl fumarate containing 0.25 percent by weight Victor 85X; and 1.5 percent by weight 2-hydroxy-4-n-octyloxybenzoylphenone. To this composition is added an additional 5 percent by weight of low density branched polyethylene (du Pont TE-4275) having a melt index of 3.7, a density of 0.923 and a melting point of 230°-250° F. The polyethylene being in fine particulate form [100 percent through a 50 mesh sieve (297 microns) and a maximum of 30 percent through a 100 mesh sieve (149 microns)]. The composition is passed through a screw extruder which reduces the mixture to a melt, and the mixture is melt extruded through a die having a plurality of rectangular openings with a 0.00225"×0.028" cross section. The molten material is pulled through an airgap of about 1 inch where partial orientation and some modification of the shape of the filament occurs. The ribbon is then passed through a water quench bath at 105° F., passed through an orientation stand including a plurality of rollers where the ratio of input to output speed is approximately 3.9:1. Subsequently, the oriented filament is passed through an annealing water bath at 205° F. at 844 feet per minute. The ribbon emerges from the annealing bath at 820' per minute and is carried onto chilled snubbing rolls.

The filaments so produced have a denier of 550, a cross section of about 2.5×28 mils a weight of 1.5 grams per denier, an elongation of 22 percent, and a shrinkage of 6 percent at 212° F. for 10 minutes.

The saran ribbon monofilament is woven together with other fibers to fabricate commercial fire-retardant draperies. These draperies, tested by an independent testing laboratory, undergo a shrinkage of only 0.5 percent after dry cleaning in perchloroethylene.

It is to be understood that the invention is not limited to the embodiment disclosed which is illustratively offered and that modifications may be made without departing from the invention.

What is claimed is:

- Extruded saran monofilament of small thickness, suitable for dry-cleanable and fire-retardant textile fabric, consisting essentially of:
    - 100 parts by weight of a copolymer of about 85 percent by weight vinylidene chloride and about 15 percent by weight vinyl chloride in which the vinyl chloride groups appear regularly spaced in the copolymer backbone without forming substantial blocks;
    - about 0.0013 to 0.0075 moles of an organic stabilizing plasticizer of an ester of fumaric acid, maleic acid, itaconic acid or aconitic acid at least a portion of said stabilizing plasticizer being joined to said copolymer by means of a Diels-Alder reaction between said plasticizer and diene portions of said copolymer backbone produced by dehydrohalogenation occurring in said copolymer dur-
  - about 0.76 to 2.65 parts by weight of an organic light stabilizer which absorbs or screens ultraviolet light; the total quantity of said organic light stabilizer and said organic stabilizing plasticizer being no greater than 5 percent by weight based on the total quantity of said copolymer, said stabilizer and said plasticizer;
  - about 0.16 to 0.51 parts by weight of a perchloroethylene nonextractable, primarily inorganic phosphate stabilizer; and
  - about 3 to 9 parts by weight of branched polyethylene.
2. An extruded saran monofilament in accordance with claim 1 of rectangular cross section having a thickness of about 2 to 2.5 mils and a width of about 25-30 mils.
3. An extruded saran monofilament in accordance with claim 2 wherein said polyethylene is present in an amount of about 5 percent by weight, said polyethylene having a melt index of about 3.7, a density of about 0.923 and a melting point in the range of 230°-250° F.
4. An extruded saran monofilament in accordance with claim 2 wherein said organic stabilizing plasticizer is present in an amount of 0.0045 to 0.0075 moles.
5. An extruded saran monofilament in accordance with claim 2, wherein said organic stabilizing plasticizer is diethyl fumarate and is present in an amount of about 2.5 percent by weight based on the composition exclusive of the polyethylene.
6. An extruded saran monofilament in accordance with claim 2, wherein said organic light stabilizer is 2,4-dibenzoyl-resorcinol or a 2-hydroxy-4-n-alkyloxybenzophenone, wherein the alkyl consists of up to 18 carbon atoms.
7. An extruded saran monofilament in accordance with claim 2, wherein said organic light stabilizer is 2-hydroxy-4-n-octyloxybenzophenone and is present in an amount of about 1.5 percent by weight based on the composition exclusive of the polyethylene.
8. An extruded saran monofilament in accordance with claim 2, wherein said perchloroethylene nonextractable, primarily inorganic stabilizer is disodium phosphate, sodium pentacapryl tripolyphosphate, sodium tripolyphosphate, tetrasodium pyrophosphate, sodium hexametaphosphate, sodium barium pyrophosphate, barium stearyl phosphate, barium lauryl phosphate, sodium metaphosphate or mixtures thereof.
9. An extruded saran monofilament in accordance with claim 2 wherein said perchloroethylene nonextractable, primarily inorganic stabilizer consists of a blend of about 88 percent by weight disodium phosphate and about 12 percent by weight of sodium pentacapryl tripolyphosphate, said blend being present in an amount of about 0.25 percent by weight based on the composition exclusive of the polyethylene.
10. An extruded saran monofilament in accordance with claim 2 comprising 95.75 percent by weight of said copolymer; 2.5 percent by weight of said organic stabilizing plasticizer which consists of diethyl fumarate; 1.5 percent by weight of said organic light stabilizer which consists of 2-hydroxy-4-n-octyloxybenzophenone; 0.25 percent by weight of said perchloroethylene nonextractable, primarily inorganic stabilizer which consists of a blend of 88 percent by weight of disodium phosphate and 12 percent by weight of sodium pentacapryl tripolyphosphate; and an additional 5 percent by weight of said branched polyethylene.

ing extrusion thereof;

15

e. about 3 to 9 parts by weight of branched polyethylene.

2. An extruded saran monofilament in accordance with claim 1 of rectangular cross section having a thickness of about 2 to 2.5 mils and a width of about 25-30 mils.

3. An extruded saran monofilament in accordance with claim 2 wherein said polyethylene is present in an amount of about 5 percent by weight, said polyethylene having a melt index of about 3.7, a density of about 0.923 and a melting point in the range of 230°-250° F.

4. An extruded saran monofilament in accordance with claim 2 wherein said organic stabilizing plasticizer is present in an amount of 0.0045 to 0.0075 moles.

5. An extruded saran monofilament in accordance with claim 2, wherein said organic stabilizing plasticizer is diethyl fumarate and is present in an amount of about 2.5 percent by weight based on the composition exclusive of the polyethylene.

6. An extruded saran monofilament in accordance with claim 2, wherein said organic light stabilizer is 2,4-dibenzoyl-resorcinol or a 2-hydroxy-4-n-alkyloxybenzophenone, wherein the alkyl consists of up to 18 carbon atoms.

7. An extruded saran monofilament in accordance with claim 2, wherein said organic light stabilizer is 2-hydroxy-4-n-octyloxybenzophenone and is present in an amount of about 1.5 percent by weight based on the composition exclusive of the polyethylene.

8. An extruded saran monofilament in accordance with claim 2, wherein said perchloroethylene nonextractable, primarily inorganic stabilizer is disodium phosphate, sodium pentacapryl tripolyphosphate, sodium tripolyphosphate, tetrasodium pyrophosphate, sodium hexametaphosphate, sodium barium pyrophosphate, barium stearyl phosphate, barium lauryl phosphate, sodium metaphosphate or mixtures thereof.

9. An extruded saran monofilament in accordance with claim 2 wherein said perchloroethylene nonextractable, primarily inorganic stabilizer consists of a blend of about 88 percent by weight disodium phosphate and about 12 percent by weight of sodium pentacapryl tripolyphosphate, said blend being present in an amount of about 0.25 percent by weight based on the composition exclusive of the polyethylene.

10. An extruded saran monofilament in accordance with claim 2 comprising 95.75 percent by weight of said copolymer; 2.5 percent by weight of said organic stabilizing plasticizer which consists of diethyl fumarate; 1.5 percent by weight of said organic light stabilizer which consists of 2-hydroxy-4-n-octyloxybenzophenone; 0.25 percent by weight of said perchloroethylene nonextractable, primarily inorganic stabilizer which consists of a blend of 88 percent by weight of disodium phosphate and 12 percent by weight of sodium pentacapryl tripolyphosphate; and an additional 5 percent by weight of said branched polyethylene.